

1  
2,774,691TREATMENT OF TEXTILE MATERIALS AND  
PRODUCT

Carl W. Schroeder, Orinda, and Robert W. Sumers, Berkeley, Calif., assignors to Shell Development Company, New York, N. Y., a corporation of Delaware

No Drawing. Application September 21, 1954,  
Serial No. 457,530

18 Claims. (Cl. 117—139.4)

This invention relates to the treatment of textile materials. More particularly, the invention relates to a method for treating textile materials to render them crease resistant and shrink resistant.

Specifically, the invention provides a new and highly efficient method for treating textile materials to render them crease and shrink resistant which comprises impregnating the textile fabric with an aqueous solution containing a mixture of a polyepoxide and a polyaldehyde, and an acid-acting curing catalyst and then heating the impregnated fabric to a relatively high temperature for a short period. The invention further provides improved textile fabrics prepared by the aforescribed process.

Many textile fabrics, such as those prepared from rayon and cotton, have rather poor resilience, i. e., they are easily creased or wrinkled when crushed or otherwise subjected to localized physical force. In addition, many of the fabrics have poor dimensional stability as exemplified by poor resistance to shrinkage. In order to overcome these shortcomings it has been common practice to treat the fabric with materials, such as an urea- or melamine-formaldehyde resin or glyoxal, that could be subsequently insolubilized within the fabric fibers. While these materials give some of the desired properties, they still leave much to be desired as all around crease and shrink proof agents. In some cases these materials give good wrinkle resistance but poor shrink resistance, and in other cases they give good shrink resistance but poor wrinkle resistance. In addition, many of these additives cause a permanent discoloration of the treated fabric. Others do not affect the color of the fabric initially but after the fabric has been bleached and ironed or hot-air dried, the fabric becomes charred or discolored. Still others weaken the fabrics, such as rayon, so that they have low tensile strength. Furthermore, many of the fabrics treated with these materials have a harsh feel and poor abrasion resistance.

It is an object of the invention, therefore, to provide a new method for treating textile materials. It is a further object to provide a process for preparing textile fabrics having a high degree of crease resistance and shrink resistance. It is a further object to provide a method for endowing fabrics with a high degree of both wrinkle resistance and shrink resistance without having any deleterious effect on other properties as tensile strength. It is a further object to provide a method for preparing crease and shrink resistant fabrics which are non-chlorine retentive, i. e., can be bleached and ironed without causing discoloration of the fabric. It is a further object to provide a method for rendering textile fabrics crease and shrink resistant without giving the fabrics a harsh feel and poor abrasion. Other objects and advantages of the invention will be apparent from the following detailed description thereof.

It has now been discovered that these and other objects may be accomplished by the novel process of the invention which comprises impregnating the textile fabric with an aqueous solution containing a mixture of a polyepoxide

5

20

25

30

35

40

45

50

55

60

65

70

2

and a polyaldehyde, and an acid-acting curing agent, and then heating the impregnated fabric to a relatively high temperature for a short period. It has been found that fabrics treated in this manner have unexpectedly high crease resistance as well as shrink resistance and, in fact, higher crease and shrink resistance than could be accomplished by using the same amount of either of the components separately. In addition, it has been found that these properties are obtained with little if any loss of other desired properties, such as tensile strength, which loss generally accompanies the addition of the above-noted conventional crease-proofing agents. The fabrics treated with the above-described combination also have a soft feel and good hand and excellent abrasion resistance. It has also been surprisingly found that the fabrics treated with the above mixture have no ability to retain chlorine and the treated fabrics may be bleached or otherwise exposed to chlorine without danger of being discolored, charred or weakened during subsequent heat treatment.

One of the agents employed in the treatment of the fabric according to the process of the invention is a polyepoxide. The expression polyepoxide refers to those materials possessing a plurality of epoxy, i. e.,



groups in the molecule. The polyepoxides may be saturated or unsaturated, aliphatic, cycloaliphatic, aromatic or heterocyclic and may be substituted if desired with various substituents, such as halogen atoms, hydroxyl groups, ether radicals and the like. They may also be monomeric or polymeric.

For clarity, many of the polyether polyepoxides and particularly those of the polymeric type will be described throughout the specification and claims in terms of an epoxy equivalency. The term "epoxy equivalency" as used herein has the same meaning as described in U. S. 2,633,458.

If the polyepoxide material consists of a single compound and all of the epoxy groups are intact, the epoxy equivalency will be integers, such as 2, 3, 4, and the like. However, in the case of polymeric-type polyepoxides many of the materials may contain some of the monomeric monoePOXides or have some of their epoxy groups hydrated or otherwise reacted and/or contain macromolecules of somewhat different molecular weight so the epoxy equivalency may be quite low and contain fractional values. The polymeric material may, for example, have an epoxy equivalency of 1.5, 1.8, 2.5, and the like.

Polyepoxides to be used in the process of the invention may be exemplified by 1,4-bis(2,3-epoxypropoxy)benzene, 1,3-bis(2,3-epoxypropoxy)benzene, 4,4'-bis(2,3-epoxypropoxy) diphenyl ether, 1,3-bis(2,3-epoxypropoxy)octane, 1,4-bis(2,3-epoxypropoxy)cyclohexane, 4,4'-bis(2-hydroxy-3,4-epoxybutoxy)diphenyldimethylmethane, 1,3-bis(4,5-epoxypentoxy)-5-chlorobenzene, 1,4-bis(3,4-epoxybutoxy)2-chlorocyclohexane, diglycidyl ether, ethylene glycol diglycidyl ether, resorcinol diglycidyl ether, and 1,2,3,4-tetra-(2-hydroxy-3,4-epoxybutoxy)butane.

Other examples include the glycidyl polyethers of polyhydric phenols obtained by reacting a polyhydric phenol with an excess, e. g., 4 to 8 mole excess, of a chlorohydrin, such as epichlorohydrin and dichlorohydrin. Thus, Polyether D described hereinafter, which is substantially 2,2-bis(2,3-epoxypropoxyphenyl)-propane, is obtained by reacting bis-phenol-A with an excess of epichlorohydrin in an alkaline medium. Other polyhydric phenols that can be used for this purpose include resorcinol, catechol, hydroquinone, methyl resorcinol, or polynuclear phenols,

such as 2,2-bis(4-hydroxyphenyl)butane, 4,4'-dihydroxybenzophenone, bis(4-hydroxyphenyl)ethane, and 1,5-dihydronaphthalene.

Still a further group of polyepoxides comprises the poly epoxy polyethers obtained by reacting, preferably in the presence of an acid-acting compound, such as hydrofluoric acid, one of the aforescribed halogen-containing epoxides with a polyhydric alcohol, and subsequently treating the resulting product with an alkaline component. As used herein and in the claims, the expression "polyhydric alcohol" is meant to include those compounds having at least two free alcoholic OH groups and includes the polyhydric alcohols and their ethers and esters, hydroxy-aldehydes, hydroxyketones, halogenated polyhydric alcohols, and the like. Polyhydric alcohols that may be used for this purpose may be exemplified by glycerol, propylene glycol, ethylene glycol, diethylene glycol, butylene glycol, hexanetriol, sorbitol, mannitol, pentaerythritol, polyallyl alcohol, polyvinyl alcohol, inositol, trimethylolpropane, bis(4-hydroxycyclohexyl)dimethylmethane, 1,4-dimethylolbenzene, 4, 4'-dimethyloldiphenyl, dimethyloltoluenes, and the like. The polyhydric ether alcohols include, among others, diglycerol, triglycerol, dipentaerythritol, tripentaerythritol, dimethylolanisoles, beta-hydroxyethyl ethers of polyhydric alcohols, such as diethylene glycol, polyethylene glycols, bis(beta-hydroxyethyl ether) of hydroquinone, bis(beta-hydroxyethyl ether) of bisphenol, beta-hydroxyethyl ethers of glycerol, pentaerythritol, sorbitol, mannitol, etc., condensates of alkylene oxides, such as ethylene oxide, propylene oxide, butylene oxide, isobutylene oxide, glycidyl, epichlorohydrin, glycidyl ethers, etc., with polyhydric alcohols, such as the foregoing and with polyhydric thioethers, such as 2,2'-dihydroxydiethyl sulfide, 2,2'-3,3'-tetrahydroxy dipropyl sulfide, etc. The hydroxylaldehydes and ketones may be exemplified by dextrose, fructose, maltose, glyceraldehyde. The mercapto (thiol) alcohols may be exemplified by alpha-monothioglycerol, alpha, alpha-dithioglycerol, etc. The polyhydric alcohol esters may be exemplified by monoglycerides, such as monostearin, monoesters of pentaerythritol and acetic acid, butyric acid, pentanoic acid, and the like. The halogenated polyhydric alcohols may be exemplified by the monochloride of pentaerythritol, monochloride of sorbitol, monochloride of mannitol, monochloride of glycerol, and the like.

A further group of the polyepoxides comprise the polyepoxy polyesters obtained by esterifying a polycarboxylic acid with an epoxy-containing alcohol, such as, for example, the diglycidyl esters of polycarboxylic acids as diglycidyl phthalate, diglycidyl maleate, diglycidyl adipate and the like.

Other polyepoxides include the polyepoxypolyhydroxy polyethers obtained by reacting, preferably in an alkaline medium, a polyhydric alcohol or polyhydric phenol with a polyepoxide, such as the reaction product of a glycidyl ether of a polyhydric phenol with the same or different polyhydric phenol, the reaction product of glycerol and bis(2,3-epoxypropyl) ether, the reaction product of sorbitol and bis(2,3-epoxy-2-methylpropyl) ether, the reaction product of pentaerythritol and 1,2-epoxy-4,5-epoxypentane, and the reaction product of bis-phenol and bis(2,3-epoxy-2-methylpropyl) ether, the reaction product of resorcinol and bis(2,3-epoxypropyl) ether, and the reaction product of catechol and bis(2,3-epoxypropyl) ether.

A group of polymeric-type polyepoxides comprises the hydroxy-substituted polyepoxide polyethers obtained by reacting, preferably in an alkaline medium, a slight excess, e. g., 5 to 3 mole excess, of a halogen-containing epoxide, such as epichlorohydrin, with any of the aforescribed polyhydric phenols, such as resorcinol, catechol, 2,2-bis(4'-hydroxyphenyl)propane, bis[4-(2'-hydroxynaphthyl)-2-2-hydroxynaphthyl] methane, and the like.

Other polymeric polyepoxides include the polymers and copolymers of the allylic ether of epoxy-containing alcohols. When this type of monomer is polymerized in the substantial absence of alkaline or acidic catalysts, such as in the presence of heat, oxygen, peroxy compounds, actinic light, and the like, they undergo additional polymerization at the multiple bond leaving the epoxy group unaffected. These allylic ethers may be polymerized with themselves or with other ethylenically unsaturated monomers, such as styrene, vinyl acetate, methacrylonitrile, acrylonitrile, vinyl chloride, vinylidene chloride, methyl acrylate, methyl methacrylate, diallyl phthalate, vinyl allyl phthalate, divinyl adipate, 2-chloroallyl acetate, and vinyl methallyl pimelate. Illustrative examples of these polymers include poly(allyl 2,3-epoxypropyl ether), allyl 2,3-epoxypropyl ether-styrene copolymer, methallyl 3,4-epoxybutyl ether-allyl benzoate copolymer, poly(vinyl-2,3-epoxypropyl)ether and an allyl glycidyl ether-vinyl acetate copolymer.

Coming under special consideration are the polyglycidyl polyethers of polyhydric alcohols obtained by reacting the polyhydric alcohol with epichlorohydrin, preferably in the presence of 0.1% to 5% by weight of an acid-acting compound, such as boron trifluoride, hydrofluoric acid, stannic chloride or stannic acid. This reaction is effected at about 50° C. to 125° C. with the proportions of reactants being such that there is about one mole of epichlorohydrin for every equivalent of hydroxyl group in the polyhydric alcohol. The resulting chlorohydrin ether is then dehydrochlorinated by heating at about 50° C. to 125° C. with a small, e. g., 10% stoichiometrical excess of a base such as sodium aluminate.

The products obtained by the method shown in the preceding paragraph may be described as polyether polyepoxide reaction products which in general contain at least three non-cyclic ether (—O—) linkages, terminal epoxide-containing ether



groups and halogen attached to a carbon of an intermediate



group.

These halogen-containing polyether polyepoxide reaction products obtainable by partial dehydrohalogenation of polyhalohydrin alcohols may be considered to have the following general formula



in which R is the residue of the polyhydric alcohol which may contain unreacted hydroxyl groups, X indicates one or more of the epoxy ether groups attached to the alcohol residue, y may be one or may vary in different reaction products of the reaction mixture from zero to more than one, and Z is one or more, and X+Z, in the case of products derived from polyhydric alcohols containing three or more hydroxyl groups, averages around two or more so that the reaction product contains on the average two or more than two terminal epoxide groups per molecule.

The preparation of one of these preferred polyglycidyl ethers of polyhydric alcohols may be illustrated by the following example showing the preparation of a glycidyl polyether of glycerol.

PREPARATION OF GLYCIDYL POLYETHERS  
OF POLYHYDRIC ALCOHOLS

## Polyether A

About 276 parts (3 moles) of glycerol was mixed with 832 parts (9 moles) of epichlorohydrin. To this reaction mixture was added 10 parts of diethyl ether solution containing about 4.5% boron trifluoride. The temperature of this mixture was between 50° C. and 75° C. for about 3 hours. About 370 parts of the resulting glycerol-epichlorohydrin condensate was dissolved in 900 parts of dioxane containing about 300 parts of sodium aluminate. While agitating, the reaction mixture was heated and refluxed at 93° C. for 9 hours. After cooling to atmospheric temperature, the insoluble material was filtered from the reaction mixture and low boiling substances removed by distillation to a temperature of about 150° C. at 20 mm. pressure. The polyglycidyl ether, in amount of 261 parts, was a pale yellow viscous liquid. It had an epoxy value of 9.671 equivalent per 100 grams and the molecular weight was 324, as measured ebullioscopically in dioxane solution. The epoxy equivalency of this product was 2.13. For convenience, this product will be referred to hereinafter as Polyether A.

## Polyether B

10.5 moles of ethylene oxide was bubbled through 3.5 moles glycerine containing an acid catalyst at 40-50° C. The resulting product had a molecular weight of 224 and a hydroxyl value of 1.417 eq./100 g. 101 parts of this ethylene oxide glycerine condensate was placed in a reaction kettle and heated to 65-70° C. Sufficient  $\text{BF}_3$ -Ethyl ether complex was added to bring the pH to about 1.0 and then 132 parts of epichlorohydrin added dropwise. After all the epi had been added, the reaction was continued for about 15 minutes to assure complete reaction. This product was then dissolved in benzene and 57 parts of sodium hydroxide were added in 7 equal portions at about 87-89° C. over a period of 3/4 hour and then filtered to remove the salt. The solvent and light ends were then removed by stripping at a low vacuum. The resulting product had a molecular weight of 455, and an epoxy value of .524 eq./100 g. For convenience, this polyether will be referred to herein as Polyether B.

## Polyether C

One equivalent of 1,2,6-hexanetriol was placed in a reaction kettle and heated to 65-70° C. Sufficient  $\text{BF}_3$ -Ethyl ether complex was added to bring the pH to about 1.0 and then 1 equivalent of epichlorohydrin added dropwise. After all the epi had been added, the reaction was continued for about 15 minutes to assure complete reaction. This product was then dissolved in acetone and sodium orthosilicate was added at about 65° C. over a period of 0.5 hour and then filtered to remove the salt. The solvent and light ends were then removed by stripping at a low vacuum. The resulting product had a molecular weight of 325 and an epoxy value of .600 eq./100 g. For convenience, this polyether will be referred to herein as Polyether C.

Particularly preferred members of this group comprise the glycidyl polyethers of aliphatic polyhydric alcohols containing from 2 to 10 carbon atoms and having from 2 to 6 hydroxyl groups and more preferably the alkane polyols containing from 2 to 8 carbon atoms and having from 2 to 6 hydroxyl groups. Such products preferably have an epoxy equivalency greater than 1.0, and still more preferably between 1.1 and 4 and a molecular weight between 300 and 1000.

Also of importance are the monomeric and polymeric glycidyl polyethers of dihydric phenols obtained by reacting epichlorohydrin with a dihydric phenol in an alkaline medium. The monomeric products of this type may be represented by the general formula



wherein R represents a divalent hydrocarbon radical of the dihydric phenol. The polymeric products will generally not be a single simple molecule but will be a complex mixture of glycidyl polyethers of the general formula



wherein R is a divalent hydrocarbon radical of the dihydric phenol and n is an integer of the series 0, 1, 2, 3, etc. While for any single molecule of the polyether n is an integer, the fact that the obtained polyether is a mixture of compounds causes the determined value of n to be an average which is not necessarily zero or a whole number. The polyethers may, in some cases, contain a very small amount of material with one or both of the terminal glycidyl radicals in hydrated form.

The aforescribed preferred glycidyl polyethers of the dihydric phenols may be prepared by reacting the required proportions of the dihydric phenol and the epichlorohydrin in an alkaline medium. The desired alkalinity is obtained by adding basic substances, such as sodium or potassium hydroxide, preferably in stoichiometric excess to the epichlorohydrin. The reaction is preferably accomplished at temperatures within the range of from 50° C. to 150° C. The heating is continued for several hours to effect the reaction and the product is then washed free of salt and base.

The preparation of some of the glycidyl polyethers of the dihydric phenols will be illustrated below.

## 30 PREPARATION OF GLYCIDYL POLYETHERS OF DIHYDRIC PHENOLS

## Polyether D

About 2 moles of bis-phenol was dissolved in 10 moles of epichlorohydrin and 1% to 2% water added to the resulting mixture. The mixture was then brought to 80° C. and 4 moles of solid sodium hydroxide added in small portions over a period of about 1 hour. During the addition, the temperature of the mixture was held at about 90° C. to 110° C. After the sodium hydroxide had been added, the water formed in the reaction and most of the epichlorohydrin was distilled off. The residue that remained was combined with an approximately equal amount of benzene and the mixture filtered to remove the salt. The benzene was then removed to yield a viscous liquid having a viscosity of about 150 poises at 25° C. and a molecular weight of about 350 (measured ebullioscopically in ethylene dichloride). The product had an epoxy value of 0.50 eq./100 g., and an epoxy equivalency of 1.75. For convenience, this product will be referred to hereinafter as Polyether D.

Particularly preferred members of the above-described group are the glycidyl polyethers of the dihydric phenols, and especially 2,2-bis(4'-hydroxyphenyl) propane, having an epoxy equivalency between 1.1 and 2.0 and a molecular weight between 300 and 900. Particularly preferred are those having a Durrans' Mercury Method softening point below about 60° C.

The glycidyl polyethers of polyhydric phenols obtained by condensing the polyhydric phenols with epichlorohydrin are also referred to as "ethoxylene" resins. See Chemical Week, vol. 69, page 27, for September 8, 1951.

Of particular value in the process of the invention are the polyepoxides containing only carbon, hydrogen, oxygen and halogen atoms.

The polyaldehydes to be used in combination with the above-described polyepoxides comprise those organic materials possessing a plurality of aldehyde, i. e.,



These materials may be saturated or unsaturated, aliphatic, cycloaliphatic aromatic or heterocyclic and substituted with substituents, such as alkoxy radicals, halogen atoms, ester radicals and the like. Examples of

these polyaldehydes include, among others, glyoxal, glutaraldehyde, adipaldehyde, pimelaldehyde, suberaldehyde, glutaconaldehyde, alphahydroxyadipaldehyde, beta-methoxyadipaldehyde, alpha,gamma - dimethyl - alpha-(methoxymethyl) glutaraldehyde, beta-allyloxy-pimelaldehyde, 1,4-cyclohexandicarboxaldehyde, 3-cyclohexene-1,5 - dicarboxaldehyde, 1,1,5 - pentanetricarboxaldehyde and 1,3,6-octane-tricarboxaldehyde.

A preferred group of polyaldehydes comprise glyoxal, succinaldehyde, glutaraldehyde and hydrocarbyl-substituted glutaraldehydes, such as those of the formula



wherein each R is hydrogen or an alkyl, cycloalkyl, alkenyl, cycloalkenyl, aryl, alkaryl or an aralkyl group. Examples of these dialdehydes include beta-methyl-glutaraldehyde, beta,gamma-dibutylglutaraldehyde, beta-phenylglutaraldehyde, beta,gamma - dibenzylglutaraldehyde, beta,gamma-dicyclohexylglutaraldehyde, and beta-isopropylphenylglutaraldehyde. A detailed description of how to prepare these glutaraldehydes may be found in Smith et al., U. S. 2,546,018.

Another preferred group of polyaldehydes comprise the ether-substituted dialdehydes, such as those obtained by reacting a suitable alpha-methylene monoaldehyde, such as methacrolein, with an alcohol under controlled conditions and in the presence of a basic condensation catalyst. The over-all reaction which is effected in the execution of this process may be exemplified by the following equation:



In this equation, ROH signifies an alcohol containing the organic radical R which is preferably a hydrocarbon radical, and R<sub>1</sub> represents a hydrocarbon group, preferably an alkyl, cycloalkyl, aryl, alkaryl or aralkyl group. For example when R is allyl and R<sub>1</sub> represents methyl, the product is alpha,gamma-dimethyl-alpha-(allyloxymethyl) glutaraldehyde. Other examples of these preferred aldehydes include alpha, gamma-dimethyl-alpha(methoxymethyl) glutaraldehyde, alpha,gamma-dimethyl-alpha-(propoxymethyl) glutaraldehyde, alpha,gamma-dimethyl-alpha-(hydroxyethoxymethyl) glutaraldehyde, alpha,gamma-dimethyl-alpha-(hydroxyethoxymethyl) glutaraldehyde, alpha,gamma-dimethyl-alpha-(methallyloxymethyl) glutaraldehyde, alpha,gamma-dicyclohexyl - alpha-(methallyloxymethyl) glutaraldehyde, alpha,gamma - dibutyl - alpha-(dodecylloxymethyl) glutaraldehyde, and alpha,gamma-dioctyl-alpha-(octadecenylloxymethyl) glutaraldehyde. Especially preferred members of this group are those of the formula:



wherein R is a hydrocarbon or hydroxy-substituted hydrocarbon radical, and particularly an alkyl, alkenyl, cycloalkyl or cycloalkenyl radical and their hydroxy-substituted derivatives, and R<sub>1</sub> is an alkyl, alkenyl cycloalkyl or cycloalkenyl radical, wherein 11 of the foregoing radicals preferably contain no more than 8 carbon atoms. A detailed description of the method for preparing the above-described preferred polyaldehydes may be found in copending patent application of Smith and Norton, Serial No. 16,617, filed March 23, 1948.

Another preferred group of polyaldehydes comprise the hydroxy-substituted dialdehydes and particularly the alpha-hydroxy-substituted adipaldehydes, such as, for example, alpha-hydroxy-adipaldehyde, alpha-hydroxy-gamma, delta-dimethyladipaldehyde, alpha-hydroxy-gamma-ethyl-delta-isopropyl-adipaldehyde, and alpha-hydroxy-gamma-delta-dioctyladipaldehyde. A detailed description for preparing some of these polyaldehydes from

substituted dihydro-1,4-pyrans may be found in Whetstone et al.—U. S. 2,639,297.

Another group of preferred polyaldehydes comprise those obtained by condensation of methacrolein in the presence of aqueous alkali as described in J. Am. Chem. Soc. 60, 1737 and 1911 (1938), and polyaldehydes obtained by condensing acrolein with alcohols in the presence of a basic catalyst as described in German Patent 554,949.

Still another group of preferred polyaldehydes comprise the polymers and copolymers obtained by polymerizing unsaturated aldehydes. Examples of such unsaturated aldehydes include, among others, acrolein, alpha-methyl acrolein, alpha-ethyl acrolein, alpha-propyl acrolein, alpha-isobutyl acrolein, alpha-n-amy1 acrolein, alpha-n-hexyl acrolein, alpha-bromo acrolein, crotonaldehyde, alpha-chloro-crotonaldehyde, alpha-bromo-crotonaldehyde, alpha-beta-dimethylacrolein, alpha-methyl-beta-ethyl acrolein, alpha-ethyl-beta-propylacrolein, and the like. Preferred unsaturated aldehydes to be used in preparing these polymers include the alpha,beta-ethylenically unsaturated aldehydes, and particularly the 2-alkenals containing no more than 8 carbon atoms.

Monomers that can be copolymerized with the above-described unsaturated aldehydes to form polyaldehydes comprise those compounds containing a polymerizable unsaturated linkage, and preferably a single  $\text{CH}_2=\text{C}=$  group, such as, for example, styrene, alpha-methyl styrene, vinyl chloride, vinylidene chloride, methyl methacrylate, ethyl acrylate, acrylonitrile, methacrylonitrile, allyl acetate, vinyl acetate, chloroallyl caproate, allyl alcohol, isobutylene, allyl glycidyl ether, vinyl methyl ether, allyl glycolate, methyl allyloxy-acetate, vinyl pyridine, glycidyl methacrylate, hydroxyethyl methacrylate, octyl acrylate, vinyl pyrrolidone, allyl dimethyl cyanurate, allyl butyl phthalate, dialkyl maleates, and the like. In preparing copolymers of the unsaturated aldehydes with these dissimilar monomers it is preferred to employ the dissimilar monomer in amounts varying from 1% to 70% by weight of the total monomer mixture.

The ratio in which the polyepoxide and the polyaldehyde are combined in the mixture may vary within certain limits. At least 15% by weight and preferably from 15% to 90% by weight of the mixture should be made up of the polyepoxide and the remainder being the polyaldehyde. The highest wrinkle resistance and shrink resistance, however, are generally obtained when the polyepoxide varies from 30% to 70% by weight and the remainder being the polyaldehyde.

The polyepoxide and the polyaldehyde are applied to the fabric in the form of an aqueous solution. Many of the polyaldehydes and polyepoxides will be water soluble and the aqueous solutions may be prepared by merely adding the mixture of polyaldehyde and polyepoxide to the water. In other cases, it may be helpful to add solvents, such as acetone, ethyl alcohol and dioxane to the water, or to employ emulsifying agents to assist in the formation of the water solution. If emulsifying agents are employed, they are preferably those that are free of nitrogen and strong acidic groups, such as the monooleate of sorbitan polyoxyethylene, the trioleate of sorbitan polyoxyethylene, sorbitan tristearate, sorbitan monolaurate, polyoxyethylene esters of alkylphenols, carboxymethylcellulose, starch, gum arabic, polyvinyl alcohol, aryl and alkylated aryl sulfonates, such as cetyl sulfonate, oleyl sulfonate, sulfonated mineral oils, copolymers of vinyl methyl ether, maleic anhydride and the like, and mixtures thereof. The emulsifying agents are generally employed in amounts varying from 0.1% to 10% by weight and more preferably from 1% to 5% by weight.

The amount of the mixture of polyepoxide and polyaldehyde to be employed in the impregnating solution will vary depending chiefly on the amount of the mixture to be deposited on the fabric and this in turn will depend upon the number of applications and the pick-up allowed

per application. As indicated hereinafter, the amount of the mixture to be applied to the fabric will generally vary from about 3% to about 20%. If a 100% pick-up is allowed and the solution is applied but once, the impregnating solution should contain the mixture of materials in amounts varying from 3% to 20% in order to apply these same percentages to the cloth. On the other hand, if say only a 50% pick-up is allowed and the solution applied but once, the impregnating solution should contain the material in amounts varying from 6% to 40% in order to apply the material in the preferred amounts of 3% to 20%. In general applications, solution is usually applied but once with pick-ups varying from 55% to 100%.

The curing agent added to the impregnating solution is an acid-acting material. "Acid-acting" as used herein is meant to include acids as well as those materials not classified as acids but which act as such. These agents include, among others, organic and inorganic acids and their anhydrides, such as citric acid, acetic acid, acetic acid anhydride, butyric acid, caproic acid, phthalic acid, phthalic acid anhydride, tartaric acid, aconitic acid, oxalic acid, succinic acid, succinic acid anhydride, lactic acid, maleic acid, maleic acid anhydride, fumaric acid, glutaconic acid, malonic acid, acetoacetic acid, naphthalic acid, trimellitic acid, phosphoric acid, boric acid, sulfonic acid, perchloric acid, persulfuric acid, and p-toluenesulfonic acid; metal salts, such as zinc fluoborate, magnesium perchlorate, copper perchlorate, nickel fluoborate, manganese phosphate and strontium fluoborate; and amine hydrochlorides, such as hydrochlorides of aniline, benzylidene, n-propylamine, di-n-butyl amine, di-benzylamine, triethylamine, alpha-phenylethylamine, alpha-naphthylamine, beta-aminoanthraquinone, 1,3-diamino-anthraquinone, piperidine, pyridine, quinoline, morpholine, pyrrole and guanidine, and hydrochlorides of hydroxyamines as 2-amino-2-methyl propanol and isobutanol amine.

Particularly preferred curing agents to be employed are the organic and inorganic acids containing no more than 12 carbon atoms, the salts of metals having an atomic weight between 24 and 210 and inorganic acid the anion portion of which contains at least two dissimilar elements having an atomic weight above 2, such as, for example, oxalic acid, citric acid, succinic acid, zinc fluoborate, copper perchlorate, magnesium perchlorate, barium persulfate, iron perchlorate, and the like.

Coming under special consideration, particularly because of the excellent color and exceptionally fine crease proofing properties obtained therewith, are the salts of metals of groups I to IV and VIII of the periodic table of elements and inorganic acid the anion portion of which contains at least two dissimilar elements having an atomic weight above 2, and particularly inorganic acids of the formula



wherein X is a non-metal having an atomic weight above 2, Z is an element which tends to gain from 1 to 2 electrons in its outer orbit, such as oxygen and fluorine, w is an integer, y is an integer greater than 1, and a equals the valency of the radical  $(X)_w(Z)_y$ , such as sulfuric acid, fluoboric acid, fluosilicic acid, persulfuric acid, phosphoric acid and the like.

The amount of the curing agent employed will vary depending upon the type of agent selected. In general, the amount of the curing agent will vary from about 0.5% to 30% by weight of the mixture of polyaldehyde and polyepoxide. The inorganic acids are preferably employed in amounts varying from about 0.5% to 20%, the metal salts are preferably employed in amounts varying from about 1% to 15%, and the amine hydrochlorides are preferably employed in amounts varying from about 1% to 20%.

The solution employed in the treatment of the textile fabrics according to the process of the invention may also

contain plasticizers to improve the flexibility of the textiles, although these should not be present in such proportions as to render the finished materials soft or sticky at temperatures and humidities to which they may be exposed. It is found, however, that the substances employed in the present invention yield products which are sufficiently flexible for most purposes without the use of plasticizers. Among plasticizers that may be used according to the present invention may be mentioned organic and inorganic derivatives of phenols, for example, diphenylopropane and triphenyl and tricresyl phosphates, sulphonamides, alkyl phthalates, glycol phthalates, derivatives of polyhydric alcohols, such as mono-, di- and triacetin and products obtained by condensing polyhydric alcohols with themselves or with aldehydes or ketones. The compositions may also contain natural resins, e. g., shellac, and other natural resins and synthetic or semi-synthetic resins, e. g., ester gum, polyhydroxy-polybasic acid resins, phenol aldehyde and urea-aldehyde resins.

Textile softening agents may also be added in varying amounts to improve the feel of the treated fabrics. Examples of these agents include, among others, pentadecyl phenol, octadecyl succinic acid, octadecenyl succinic acid, sulfonated waxes and sulfonated alcohols, dimerized long-chain unsaturated acids, non-ionic fatty acid esters of higher polyglycerols. Preferred softeners are the epoxidized di- and triglycerides.

The application of the aqueous solution containing the polyepoxides and polyaldehydes to the textile fabric may be effected in any suitable manner, the method selected depending upon the results desired. If it is desired to apply the solution only to one surface of the material, as, for example, when it is desired to treat the back only of a fabric having a face of artificial or natural silk and a cotton back, the application may be effected by spraying or by means of rollers, or the composition may be spread upon the surface by means of a doctor blade. When, however, it is desired to coat both surfaces of the material, or if the material is to be thoroughly impregnated with it, the fabric may be simply dipped in the solution or run through conventional-type padding rollers. The solutions may also be applied locally to the material, for example, by means of printing rollers or by stenciling.

The amount of the mixture of polyepoxide and polyaldehyde to be deposited on the fabric will vary over a wide range depending upon the degree of wrinkle resistance and shrink resistance desired in the finished material. If the fabric is to have a soft feel, such as that intended for use for dresses, shirts, etc., the amount of mixture deposited will generally vary from 3% to 20% by weight of the fabric. If stiffer materials are required such as for the shoe fabrics, draperies and the like, still higher amounts of the mixture, such as of the order of 25% to 50% by weight may be deposited.

If the desired amount of mixture of polyepoxide and polyaldehyde deposited in the fabric is not obtained in one application, the solution can be applied again or as many times as desired in order to bring the amount of the mixture up to the desired level.

After the desired amount of solution has been applied to the fabric, the treated fabric is preferably dried for a short period to remove some or all of the dispersing liquid, such as water, and the like. This is generally accomplished by exposing the wet sheets to hot gas either slack or framed to dimension at temperatures ranging up to 120° C. The period of drying will depend largely on the amount of pick-up permitted during the application of the solution, and the concentration of the mixture of polyepoxide and polyaldehyde. In most instances, the drying periods of from 1 to 30 minutes should be sufficient.

The dried fabric is then exposed to relatively high temperatures to accelerate cure. Temperatures used for this purpose generally range from 100° C. to 200° C., and more preferably from 130° C. to 190° C. At these pre-

ferred temperature ranges the cure can generally be accomplished in from 1 to 10 minutes. Exposures of less than 3 minutes, e. g., 1 minute, may probably be used in continuous, commercial processing.

The process of the invention may be applied to the treatment of any textile fabric, colored or white. Such materials include the natural or artificial textile materials, such as cotton, linen, natural silk and artificial silk, such as the artificial silk obtained from cellulose acetate or other organic esters or ethers of cellulose and the regenerated cellulosic type of artificial silk obtained by the viscose, cuprammonium or nitrocellulose process, jute, hemp, rayon, animal fibers, such as wool, hair, mohair, synthetic fibers including the fibers from polyesters, such as for example the ethylene glycolterephthalic acid polyesters (Dacron), the acrylic polyvinyls, such as for example the acrylonitrile polymers (Orlon), the polyethylenes, polyurethans (Perluran), polyvinyl alcohol proteins (Caslen), Alginic (Alginic rayon), non-acrylic polyvinyls as vinyl chloride and vinylidene polymers (Vinyon), mineral fibers (Fiberglas) polyamides, such as the aliphatic dicarboxylic acid-polyamides reaction products (Nylon). While the invention has been particularly described with relation to the treatment of woven fabrics, it may also be applied to other materials, for example, knitted or netted fabrics.

The materials treated according to the process of the invention will have excellent crease resistance and improved dimensional stability and may be used for a wide variety of important applications. The woven cotton, rayon and wool fabrics, both colored and white, containing conventional amounts of resin, e. g., from 3% to 25% by weight, may be used, for example, in the preparation of soft goods, such as dresses, shirts, coats, sheets, and the like, while the fabrics containing much larger amounts of the resin, e. g., 25% to 50% may be used in other applications demanding more crispness and fullness such as the preparation of rugs, carpets, drapes, upholsteries, shoe fabrics, and the like.

To illustrate the manner in which the invention may be carried out, the following examples are given. It is to be understood, however, that the examples are for the purpose of illustration and the invention is not to be regarded as limited to any of the specific materials or conditions recited therein.

The wrinkle recovery values reported in some of the examples were determined by the Monsanto Recovery Method. The tests were carried out at 65% relative humidity and 70° F. The shrink resistance was determined by following method: The treated cloth was washed in an automatic washer using 10 parts of concentrated ammonia and 10 parts of an alkylarylpolyether alcohol (Triton X-100) for 6 minutes at 160° F. After washing, the cloth was rinsed and tumble dried for 3 minutes in a drier. The cloth was then ironed with a flat bed press without tension. The change in length of the cloth before and after this procedure was reported as the shrinkage value.

#### EXAMPLE I

(a) This example illustrates the unexpected improvement in both wrinkle resistance and shrink resistance that is obtained by using a combination of a polyepoxide and polyaldehyde on the treatment of rayon.

50 parts of Polyether A described above was combined with 5 parts of polyethylene oxide condensation product of sorbitan monopalmitate and 50 parts of a 5% solution of polyvinyl alcohol and the mixture thoroughly stirred. 100 parts of alpha-hydroxyadipaldehyde and 7.5 parts of magnesium perchlorate were then stirred into the above mixture and sufficient water added to bring the total to 1000 parts (giving a 15% solution of polyepoxide and polyaldehyde).

Rayon cloth was then impregnated with the above-described solution by means of a Butterworth-3-Roll laboratory padder. The cloth was then dried at 60° C.

for 5 minutes and cured at 160° C. for 5 minutes. The finished product was washed and rinsed three times in warm water to remove any soluble material.

The cloth treated in the above-described manner had outstanding crease and shrink resistance and these properties were obtained with little loss of tensile strength. In addition, the cloth had a soft feel, good color, improved washability and no chlorine retention.

The wrinkle recovery (average warp and fill), shrink resistance and tensile strength of the fabric treated in the above-described manner are shown in the table below:

TABLE NO. 1

| 15 | Treating agent                                      | Monsanto wrinkle recovery (avg. warp and fill) | Shrinkage (percent) | Tensile strength lbs./in. |
|----|-----------------------------------------------------|------------------------------------------------|---------------------|---------------------------|
| 20 | Mixture of polyether A and hydroxyadipaldehyde----- | 162                                            | 0.3                 | 59                        |
|    | None (control)-----                                 | 95                                             | 3.8-4.2             | 60                        |

(b) The above results are surprising and far better than could be expected by using the same amount of the 25 Polyether A or alpha-hydroxy-adipaldehyde by themselves. This is shown by the following experiment.

Solution A was prepared as follows: 150 parts of Polyether A was combined with 7.5 parts of a polyethylene oxide condensation product of sorbitan monopalmitate and 50 parts of a 5% solution of polyvinyl alcohol and the mixture thoroughly stirred. 7.5 parts of magnesium perchlorate was then stirred into the above mixture and sufficient water added to bring the total to 1000 parts.

35 Solution B was prepared as follows: 150 parts of alpha-hydroxy-adipaldehyde was combined with 7.5 parts of a polyethylene oxide condensation product of sorbitan monopalmitate and 50 parts of a 5% solution of polyvinyl alcohol and the mixture stirred. 7.5 parts of magnesium perchlorate was then stirred into the above mixture and sufficient water added to bring the total to 1000 parts.

40 Strips of rayon cloth were then impregnated with each of the above solutions by means of a Butterworth-3-Roll 45 laboratory padder. The strips were then dried at 60° C. for 5 minutes and cured at 160° C. for 5 minutes. The finished products were then washed and rinsed three times in warm water to remove any soluble material.

The wrinkle recovery (average warp and fill) and 50 shrink resistance of the strips are shown in the table below.

TABLE NO. 2

| 55 | Treating agent  | Monsanto wrinkle recovery (avg. warp and fill) | Shrinkage (percent) |
|----|-----------------|------------------------------------------------|---------------------|
| 59 | Solution A----- | 139                                            | 0.0                 |
|    | Solution B----- | 159                                            | 0.6                 |

65 From the above figures, it would be expected that the mixture of 50 parts of Polyether A and 100 parts of alpha-hydroxyadipaldehyde as used in (a) above would give only a wrinkle recovery value of about 145 and a shrink resistance of 0.45, while it actually gave a wrinkle recovery of 162 and a shrink resistance of 0.3.

#### EXAMPLE II

70 Example I (a) was repeated with the exception that the mixture employed as the crease and shrink proofing agent was made up of 100 parts of Polyether A and 50 parts of alpha-hydroxyadipaldehyde. The resulting impregnated rayon cloth had excellent crease and shrink resistance with little loss of tensile strength. In addition, the cloth had a soft feel, good color, improved wash-

## 13

ability and no chlorine retention. The wrinkle recovery value was 149 as compared to an expected value of about 145.

## EXAMPLE III

Example I (a) was repeated with the exception that the mixture employed as the crease and shrink proofing agent was made up of 75 parts of Polyether A and 75 parts of alpha-hydroxyadipaldehyde. The resulting impregnated rayon cloth had excellent crease and shrink resistance with little loss of tensile strength. In addition, the cloth had a soft feel, good color, improved washability and no chlorine retention.

## EXAMPLE IV

Example I (a) was repeated with the exception that the mixture employed as the crease and shrink proofing agent was made up of 100 parts of Polyether A and 25 parts of alpha-hydroxyadipaldehyde. The treated cloth had the same properties as the cloth shown in the preceding example.

## EXAMPLE V

This example illustrates the unexpected improvement in wrinkle recovery and shrink resistance that is obtained by using a combination of Polyether A and glyoxal with rayon.

100 parts of Polyether A was combined with .5 parts of a polyethylene oxide condensation product of sorbitan monopalmitate and 50 parts of a 5% solution of polyvinyl alcohol and the mixture thoroughly stirred. 50 parts of glyoxal and 7.5 parts of magnesium perchlorate were stirred into the above and water added to bring the total to 1000 parts.

Rayon cloth was then impregnated with the above-described solution by means of a Butterworth-3-Roll laboratory padder. The cloth was then dried at 60° C. for 5 minutes and cured at 160° C. for 5 minutes. The finished product was washed and rinsed three times in warm water to remove any soluble material.

The cloth treated in the above-described manner had excellent wrinkle resistance and shrink resistance and were obtained with little loss of tensile strength. In addition, the cloth had a soft feel, good abrasion resistance, good color and good washability. The wrinkle recovery was 152 as compared to an expected 146.

## EXAMPLE VII

This example illustrates the improvement in wrinkle recovery and shrink resistance that is obtained by using a combination of Polyether A and succinaldehyde with rayon.

About 100 parts of Polyether A and 50 parts of succinaldehyde are mixed with an acidic solution containing 540 parts of water, .25 part Methocel, 1.8 parts of a copolymer of vinyl methyl ether and maleic anhydride and .5 part of polyglycol fatty acid ester, and as the curing agent 7.5 parts of zinc fluoborate.

Rayon cloth is then impregnated with the above-described solution by means of a Butterworth-3-Roll laboratory padder. The cloth is then dried at 60° C. for 5 minutes and cured at 160° C. for 5 minutes. The finished product is then washed and rinsed three times in warm water to remove any soluble material.

The cloth treated in the above-described manner has excellent wrinkle resistance and shrink resistance and both are obtained with little loss of tensile strength. In addition, the cloth has a soft feel, good abrasion resistance, good color and good washability and no chlorine retention.

## EXAMPLE VIII

This example illustrates the unexpected improvement in wrinkle recovery and shrink resistance that is obtained by using a combination of Polyether B and alpha, gamma-dimethyl - alpha - (allyloxymethyl) glutaraldehyde with rayon.

## 14

About 75 parts of Polyether B described above and 75 parts of alpha,gamma-dimethyl-alpha-(allyloxymethyl) glutaraldehyde are mixed with an acidic solution containing 540 parts of water, .25 part Methocel, 1.8 parts of a copolymer of vinyl methyl ether and maleic anhydride and .5 part of polyglycol fatty acid ester, and as the curing agent 5 parts of citric acid.

Rayon cloth is then impregnated with the above-described solution by means of a Butterworth-3-Roll laboratory padder. The cloth is then dried at 60° C. for 5 minutes and cured at 160° C. for 5 minutes. The finished product is then washed and rinsed three times in warm water to remove any soluble material.

The cloth treated in the above-described manner has excellent wrinkle and shrink resistance and both are obtained with little loss of tensile strength. In addition, the cloth has a soft feel, good color and good abrasion resistance.

Treated cloth having related properties is obtained by replacing the Polyether B in the above-described process with equal amounts of Polyether C.

## EXAMPLE IX

This example illustrates the treatment of rayon with a mixture of Polyether D and alpha-hydroxyadipaldehyde.

About 50 parts of Polyether D and 100 parts of alpha-hydroxy-adipaldehyde are mixed with 50 parts of a polyethylene oxide condensation product of sorbitan monopalmitate and 50 parts of polyvinyl alcohol and the mixture slowly stirred together. 7.5 parts of zinc fluoborate is stirred into the mixture and then water is added to bring the total up to 1000 parts.

Rayon cloth is then impregnated with the above-described solution by means of a Butterworth-3-Roll laboratory padder. The cloth is then dried at 60° C. for 5 minutes and cured at 160° C. for 5 minutes. The finished product is then washed and rinsed three times in warm water to remove any soluble material.

The cloth treated in the above-described manner has excellent wrinkle resistance and shrink resistance and both are obtained with little loss of tensile strength. In addition, the cloth has a soft feel, good abrasion resistance, good color and good washability and no chlorine retention.

## EXAMPLE X

Examples I (a) and II to VII are repeated with the exception that the impregnating solutions are applied to cotton. The sheets of cloth treated in this manner have the same color as before the treatment, have a soft feel, good crease and shrink resistance, good washability and no chlorine retention.

We claim as our invention:

1. A process for rendering cellulosic textile fabrics crease and shrink resistant which comprises impregnating the cellulosic fabric with an aqueous solution containing a mixture of polyepoxide and an aliphatic polyaldehyde containing from 2 to 4 free



60 groups and a minor quantity of an acid-acting curing agent, and heating the resulting impregnated fabric to a relatively high temperature for a short period.

2. A process as in claim 1 wherein the fabric is rayon.  
 3. A process as in claim 1 wherein the fabric is cotton.  
 4. A process as in claim 1 wherein the acidic catalyst is a salt of (1) a metal having an atomic weight between 24 and 210, and (2) an inorganic acid the anion portion of which contains at least two dissimilar elements having an atomic weight above 2.

5. A process for rendering cellulosic textile fabrics more crease and shrink resistant which comprises impregnating the cellulosic fabric with an aqueous solution containing a mixture of (1) a glycidyl polyether of a 70 polyhydric alcohol having an epoxy equivalency between

## 15

1.1 and 3 and a molecular weight between 170 and 800, and (2) an aliphatic polyaldehyde containing from 2 to 4



groups and from .1% to 30% by weight of an acid-acting curing catalyst, and heating the resulting impregnated fabric to a temperature above 100° C. for a short period.

6. A process as in claim 5 wherein the catalyst is citric acid.

7. A process as in claim 6 wherein the catalyst is zinc fluoborate.

8. A process as in claim 6 wherein the catalyst is magnesium perchlorate.

9. A process as in claim 5 wherein the catalyst is a salt of (1) a metal of the group consisting of metals of groups I to IV and VIII of the periodic table of elements and (2) an inorganic acid of the formula



wherein X is a non-metal having an atomic weight above 2, Z is an element which tends to gain from 1 to 2 electrons in the outer orbit, w is an integer, y is an integer greater than one, and a is equal to the valency of the radical  $(\text{X})_w(\text{Z})_y$ .

10. A process as in claim 5 wherein the polyepoxide is a glycidyl polyether of glycerol and the polyaldehyde is alpha-hydroxy-adipaldehyde.

11. A process as in claim 5 wherein the polyepoxide is a glycidyl polyether of glycerol and the polyaldehyde is glyoxal.

12. A process as in claim 5 wherein the polyaldehyde is succinaldehyde.

## 16

13. A process as in claim 5 wherein the polyaldehyde is an alpha,gamma-dialkyl-alpha-(alkoxymethyl) glutaraldehyde.

14. A process as in claim 5 wherein the mixture of polyepoxide and polyaldehyde contains from 20% to 80% by weight of polyepoxide and the remainder is polyaldehyde.

15. A process for rendering cellulosic textile fabrics more crease and shrink resistant which comprises impregnating the cellulosic fabric with an aqueous medium containing a mixture of (1) a polyepoxide consisting of a glycidyl polyether of a polyhydric phenol wherein the polyepoxide has an epoxy equivalency greater than 1.0 and a molecular weight above 200, and (2) an aliphatic dialdehyde having from 2 to 4 aldehyde groups and not more than 15 carbon atoms, and an acid-acting catalyst, and heating the resulting fabric to a temperature above 100° C.

16. A textile fabric prepared by the process of claim 1.

17. A textile fabric prepared by the process of claim 5.

18. A textile fabric prepared by the process of claim 15.

## References Cited in the file of this patent

## UNITED STATES PATENTS

|           |          |       |               |
|-----------|----------|-------|---------------|
| 2,441,859 | Weisberg | ----- | May 18, 1948  |
| 2,512,996 | Bixler   | ----- | June 27, 1950 |
| 2,541,027 | Bradley  | ----- | Feb. 13, 1951 |
| 2,606,810 | Erickson | ----- | Aug. 12, 1952 |

## FOREIGN PATENTS

|           |        |       |              |
|-----------|--------|-------|--------------|
| 1,058,002 | France | ----- | Nov. 4, 1953 |
|-----------|--------|-------|--------------|